

July 17, 1923.

S. E. T. EWING ET AL.

1,461,977

## ORE REDUCTION

Filed Aug. 30, 1922

2 Sheets-Sheet 1



July 17, 1923.

1,461,977

S. E. T. EWING ET AL

ORE REDUCTION

Filed Aug. 30, 1922

2 Sheets-Sheet 2



Inventors  
Sidney E. T. Ewing  
Joseph L. Willey.

by Parker & Carter  
attorneys.

## UNITED STATES PATENT OFFICE.

SYDNEY EDWARD THACKER EWING AND JOSEPH LEONARD WILLEY, OF JOHANNESBURG, TRANSVAAL, SOUTH AFRICA.

## ORE REDUCTION.

Application filed August 30, 1922. Serial No. 585,291.

*To all whom it may concern:*

Be it known that we, SYDNEY EDWARD THACKER EWING and JOSEPH LEONARD WILLEY, British subjects, both residing at 5 Corner House, Commissioner Street, Johannesburg, Transvaal Province, Union of South Africa, have invented certain new and useful Improvements in Ore Reduction, of which the following is a specification.

10 The present invention has reference to the reduction of ores, and especially gold ores, by processes involving tube-milling.

In the usual methods of reducing gold ores the tube mill performs the function of 15 fine grinding a product which has already been successively reduced firstly by rock breakers and secondly by stamps or ball mills (in which metal balls are used as the grinding charge). The stamp or ball mill 20 product varies in size from 200 mesh up to  $\frac{1}{4}$  inch, or in some cases 1 inch, mesh and its individual fragments are of generally cubical form without sharp angularities.

In order to effect the reduction of this 25 stamp or ball mill product in the tube mill, it is necessary to feed into the tube mill, with said product, a proportion of large pebbles which are usually pieces of ore selected from the ore stream before the latter 30 reaches the breakers. They average in size from 6 to 7 inch cubes and are added in the proportion of usually five to seven per cent of the regular mill feed, i. e., the stamp or ball mill product. The tube mill effluent is 35 commonly divided into three products namely (1) fine sand and slime which is the finished product, (2) coarse sand which is insufficiently reduced and (3) so called "reject pebbles." The first two products 40 represent the original mill feed in a more comminuted form, together with so much of the grinding charge as has become comminuted to their grade. The coarse sand is returned by the classifiers to the tube mill 45 feed, so that the original tube mill feed remains in the tube mill circuit until it is fully comminuted. The third product, namely, the "reject pebbles," consists of elements of the original grinding charge which 50 on account of their roundness and relatively small size have become inefficient for grinding purposes. If they are of ore material, they are recovered and crushed, e. g., in the

stamp mill, to the regular tube mill feed size and mingled with the feed to the tube 55 mill.

The present invention is a method of operating with a tube mill whereby on the one hand the ratio of reduction within the same is increased and on the other hand a higher 60 percentage of finished pulp in the tube mill circuit effluent is obtained without that decrease in the rate of feeding which would be necessary to effect the same result under present practice. This renders feasible and 65 economical a process of ore reduction which involves the use of the tube mill and pebble crackers assisted or not by rock breakers, obviates the necessity of the stamp mill, ball mill, disc crusher, rolls or other crushing 70 appliances hitherto deemed necessary to make a product suitable for tube-milling; and by the economical production of a one product pulp with its concomitant advantage of simplified treatment, makes possible, 75 in many cases, the elimination of the processes of amalgamation and sand treatment.

The invention consists in a method of ore reduction involving the use of a tube mill in which the regular tube mill feed 80 material consists of,—or contains,—a large proportion of large and angular fragments of ore; and in which constituent pieces of such feed material which have become rounded and therefore inefficient for comminution, are withdrawn from the tube mill, broken to make an angular product, 85 and returned to the mill.

The large and angular ore fragments which it is proposed thus to feed to the mill 90 are best represented by those present in run of mine gold ore; and the invention contemplates feeding run of mine ore directly to the tube mill in appropriate cases; in which event the whole of the reduction is effected 95 by the tube mill, supplemented by the reject pebble cracker. As however the size of material which can be economically fed to a tube mill depends upon the size and proportions of the mill itself, it is desirable in many 100 cases and is within the scope of the invention, to break the larger pieces of rock before they are fed to the mill. If the larger pieces are thus broken, it is usually desirable to feed to the mill a proportion of selected pebbles, as in the ordinary practice. 105

- It appears that as the result of thus feeding large and angular ore fragments as the regular tube mill feed, instead of stamp or ball mill product, a material modification of the reduction process within the mill is brought about. Whilst doubtless a considerable amount of reduction is done by the progressive division by fracture of individual pieces into smaller and smaller pieces, there is clear evidence that a greater part than hitherto is taken by the attrition of the angular prominences of the larger pieces. This appears to effect comminution at a rapid rate until the angularities disappear, when the resulting rounded pebbles become an inert constituent of the charge and if allowed to accumulate would seriously reduce the capacity of the mill. The systematic withdrawal of these rounded pebbles so that they may be broken and again made angular is therefore an important feature of this invention. In this respect there is an essential difference from the withdrawal of reject pebbles in the present practice, where they are the residue of the added grinding charge, the mill feed material being left in the tube mill circuit until it is reduced, at least to sand. The present method marks a distinct departure by withdrawing tube mill feed in pieces of such size as still to be capable of being broken in a rock breaker; and this is the only product which, in carrying out the invention, necessarily requires to be thus broken.
- The functions of the added pebbles in the present case are probably different from the grinding function which they exercise in a mill fed with stamp mill or ball mill product; and is rather that of securing effective relative rotation of the elements of the charge.

In the accompanying drawings:—

Figs. I and II are respectively an elevation and plan showing diagrammatically a plant for carrying out the invention.

Fig. III is a vertical section of the discharge end of the tube mill,

Fig. IV is a face view of the discharge screen therefor and

Fig. V is a sectional view of the tube mill inlet trunnion and feed hopper.

The plant shown is one employing a usual standard size of tube mill, namely, 22 feet long by 5 feet 6 inches diameter, which renders desirable the preliminary breaking of the larger pieces of ore. Accordingly ore is delivered from the shaft bins 1 to the grizzly 2. The grizzly undersize is taken direct to the tube mill ore bin 3 which feeds the tube mill 4. The grizzly oversize goes to a single stage breaker 5 and the broken product is taken, with the grizzly undersize, to the ore bin 3. The selected pebbles are in the usual manner withdrawn from the breaker feed and sent to the pebble bin 6 for supply to

the tube mill; the quantity being as a rule 8 to 10 per cent of the total fresh material passed into the tube mill.

The material thus delivered to the tube mill bin 3, namely, the grizzly undersize and the single stage breaker product, is, as regards the form of its constituent pieces, adapted for self-communition in the mill, in that besides being distinctively angular it also contains a considerable proportion of slabby fragments.

As regards the size of this material, we have found that a product passing through grizzlies set at three quarters of an inch apart, together with a corresponding breaker product, is about the least that is efficiently self-communitioning in the tube mill. The degree by which this lower limit may be exceeded depends upon the proportion of the reduction which can economically be allocated to the breaker and the tube mill respectively and would be determined largely by the dimensions of the tube mill which it is proposed to use in any particular case. We have found that when using a tube mill of the dimensions stated above economical results with ore from the deep level mines of the Far East Witwatersrand area have been attained when the material varies from  $\frac{3}{4}$  inch to  $1\frac{1}{4}$  inch grizzly product.

The usual arrangements for feeding stamp mill or ball mill pulp into the tube mill are not suitable for passing in the large dry fragments contemplated by this invention. We have found however that the difficulty can be overcome by using a hopper 7 opening into the inlet trunnion 8 of the tube mill 4 and having a steeply sloping back 9; and making the trunnion 8 of greater internal diameter than is usual. Said hopper 7 receives the ore from the bin 3, the selected pebbles from the bin 6, and the sand from the classifier 10. If grinding in cyanide is adopted the strong cyanide solution may also be added at this point.

The tube mill discharge arrangements are such as to withdraw from the outlet end of the mill a very much higher proportion than hitherto of large material; in fact we have found it desirable to withdraw the whole product from the discharge end of the mill as rapidly as is consistent with maintaining the proper level of the load in the mill. To accomplish this there is provided an outlet screen 11 which is extensively perforated with large apertures 12; preferably slots about  $1\frac{1}{4}$  inches wide and 6 inches long. There are also provided scoops 13 which at once discharge into the outlet trunnion 14 all material which passes through the screen.

The usual devices are employed for separating the tube mill effluent into the desired constituents. Sand and slime passing through the revolving screen 15 into the

launder 16 are conducted thereby to the classifier 10 which separates the coarse sand from the finished product and passes the sand to the hopper 7.

5. The single final product from the classifier 10 is shown as being conducted directly to the slime plant 17.

The reject pebbles pass along the screen 15 and are carried by the belt 18 to the pebble cracker 19, the product from which passes to the ore bin 3.

As mentioned above reject pebbles are removed in much greater quantity than hitherto; and we have found it possible and advantageous to remove, in this form, from ten per cent upwards of the total fresh material fed to the mill as compared with  $\frac{1}{2}$  to 2 per cent under present practice. With the particular ores referred to above, we regularly remove 18 to 21 per cent, and the proportion may be increased with appropriate ore and size of feed material.

In the absence of the stamp mill, the pebble cracker 19 constitutes an additional unit of the plant rendered necessary by the new process, and to a certain extent it may be regarded as a secondary crusher, but its function is more economically performed than that of the ordinary secondary crusher 20 in a stage crushing plant inasmuch as its position in the plant necessitates its operating merely on the residue of material which has ceased to be efficiently self-comminuting.

As regards the output of the tube mill, 35 whilst the average size of the feed is increased many times, the output of fully comminuted material shows a substantial advance. For instance, with the new methods a mill of the standard dimensions stated 40 above, when treating the above mentioned ores, produced per 24 hours 145 to 155 tons of minus 90 mesh product of which 75% will pass a 200 mesh screen. It will be evident that if a coarser product is made, the 45 rate of output of the tube mill will be commensurately increased.

This product is generally suitable for immediate treatment as a slime product.

We claim—

50 1. The improvement in the art of tube-milling ore which consists in supplying to the tube mill, as the regular mill feed, ore in large and angular fragments, withdrawing from the tube mill fragments of said feed material which have become rounded, breaking them, and returning the breaker product to the tube mill.

2. The improvement in the art of tube-milling ore which consists in feeding a run 55 of mine ore to the tube mill as the regular mill feed, withdrawing from the tube mill

fragments of said feed material which have become rounded, breaking them, and returning the breaker product to the tube mill.

3. The improvement in the art of tube-milling ore which consists in supplying to the tube mill, as the regular mill feed, ore in large and angular fragments, withdrawing from the tube mill, as reject pebbles, a substantial proportion of the original material fed to the tube mill, breaking the reject pebbles and returning the breaker product to the tube mill. 65

4. The improvement in the art of tube-milling ore which consists in supplying a run of mine ore to the tube mill as the regular mill feed, withdrawing from the tube mill, as reject pebbles, a proportion of such feed, breaking the reject pebbles, and returning the breaker product to the tube mill. 70

5. The improvement in the art of tube-milling ore which consists in supplying to the tube mill, as the regular mill feed, ore in large and angular fragments, withdrawing from the mill, as reject pebbles, not less than ten per cent of the material originally fed to the tube mill, breaking the reject pebbles and returning the breaker product to the tube mill. 80

6. The improvement in the art of tube-milling ore which consists in feeding a run of mine ore to the tube mill as the regular mill feed, withdrawing from the mill as reject pebbles, not less than ten per cent of the material originally fed to the tube mill, 90 breaking the reject pebbles, and returning the breaker product to the tube mill. 95

7. The improvement in the art of tube-milling ore which consists in separating the larger pieces from a run of mine ore, breaking them in a single stage, adding the product to the remainder of the run of mine ore, feeding the whole directly to the tube mill as the regular mill feed, withdrawing from the tube mill fragments of said feed material which have become rounded, breaking them, and returning the breaker product to the tube mill. 100

8. The improvement in the art of tube-milling ore which consists in supplying thereto, as the regular mill feed, ore in large and angular fragments, withdrawing all material arriving at the discharge end of the tube mill as rapidly as is consistent with maintaining the load in the tube mill, separating pebbles from said material, breaking said pebbles, and returning the breaker product to the tube mill. 110

In testimony whereof we affix our signatures.

SYDNEY EDWARD THACKER EWING.  
JOSEPH LEONARD WILLEY.